

W. F. BLEECKER.  
PROCESS OF EXTRACTING VALUES FROM ORES.  
APPLICATION FILED MAY 24, 1912.

1,068,730.

Patented July 29, 1913.

*CL*-----*PULVERIZATION*-----

6. TREATMENT WITH SODIUM HYDROXIDE AND SODIUM CARBONATE

REMOVING SOLUTION

NEUTRALIZATION WITH ACID

VANADYL RADIUM URANYL  
CHLORIDE CHLORIDE CHLORIDE

LEACHING WITH SOLUTION OF SODIUM CARBONATE,

## WASHING AND REMOVING THE SOLUTION

Q TREATMENT WITH ACID  
VANADYL CHLORIDE (PARTLY SOLUBLE) RADIUM CHLORIDE (SOLUBLE).

### WASHING AND REMOVING SOLUTION

TREATMENT WITH SULPHURIC ACID  
VANADYL SULPHATE  
(SOLUBLE)

*i*----- REMOVING SOLUTION -----

WITNESSES  
G. D. Nottingham  
G. F. Downing

INVENTOR  
W. A. Bleecker  
By H. A. Seymour  
Attorney

# UNITED STATES PATENT OFFICE.

WARREN F. BLEECKER, OF CANONSBURG, PENNSYLVANIA, ASSIGNOR TO THE STANDARD CHEMICAL COMPANY, OF PITTSBURGH, PENNSYLVANIA.

## PROCESS OF EXTRACTING VALUES FROM ORES.

1,068,730.

Specification of Letters Patent.

Patented July 29, 1913.

Application filed May 24, 1912. Serial No. 699,595.

To all whom it may concern:

Be it known that I, WARREN F. BLEECKER, a resident of Canonsburg, in the county of Washington and State of Pennsylvania, have invented certain new and useful Improvements in Processes of Extracting Values from Ores; and I do hereby declare the following to be a full, clear, and exact description of the invention, such as will enable others skilled in the art to which it appertains to make and use the same.

This invention relates to improvements in processes for the treatment of ores, and more particularly to a process for extracting values from carnotite ores,—the object of my present invention being to provide a process for producing separate solutions predominating, respectively, in uranium, radium, and vanadium, and to so treat the ore that the amount of vanadium in the uranium and radium solutions shall be reduced to a minimum, and so that practically the entire vanadium content of the ore shall be contained in a separate solution.

A further object is to treat carnotite ores in such manner as to enhance the solubility of the radium salts.

With these and other objects in view, the invention consists in certain novel steps in the process of extracting values from ores, as hereinafter set forth and pointed out in the claims.

In the accompanying drawing, my improved process is illustrated diagrammatically.

In carrying my improved process into effect, I proceed substantially as follows:—The ore (carnotite ore for example) is first reduced to a comminuted condition in any suitable manner. The comminuted ore is first treated with a solution of an alkaline hydroxid and, if desired, an alkaline carbonate may be added to this solution. For example, sodium hydroxid and sodium carbonate may be used,—in which event, the resulting liquid product (which is withdrawn) will be a solution of sodium vanadate of the type  $Na_x(VO)_x(VO_2)_y$ , from which the vanadium may be recovered by any approved process. The ore will then be neutralized with a suitable acid. The use of sulfuric acid will preferably be avoided at this stage of the process, because it would

tend to render insoluble, the radium content of the ore. The ore will next be leached with a solution of an alkaline carbonate (such as sodium carbonate),—the temperature of such solution preferably not exceeding 90° C. This treatment will dissolve the uranium content of the ore (forming sodium uranyl carbonate,— $(Na_2CO_3)_2UO_2CO_3$ ), and as a portion of the vanadium content had been removed by the first treatment hereinbefore described, and as alkaline carbonate decomposes uranium mineral and only a small quantity of vanadium mineral, the resultant solution of the treatment with hot alkaline solution, will be very low in vanadium. This solution can be subsequently treated by any approved process for the recovery of uranium.

The first treatment of the ore with sodium hydroxid or a mixture of sodium hydroxid and sodium carbonate renders the ore low in vanadium before said ore is subjected to the leaching with hot sodium carbonate, and these two treatments also serve another important office in rendering soluble the radium content of carnotite ores, the alkaline carbonate decomposing the radium barium sulfates in the ore forming radium barium carbonate,— $RaCO_3, BaCO_3$ . The carnotite ores contain barium and sulfuric acid in quantities proportional to the formula for barium sulfate ( $BaSO_4$ ). Inasmuch as radium and barium are isomorphous, radium salts are not completely soluble in the presence of barium sulfate. The barium sulfate as well as the radium sulfate must be decomposed, (forming the carbonates) and the sodium sulfate may then be washed out. These results are attained by the treatment herein described. The ore will next be washed to free it from soluble carbonates and also sulfates originating from the radium barium sulfates above mentioned. The resultant solution will contain alkaline uranyl carbonate of the type  $(Na_2CO_3)_2UO_2CO_3$ , and alkaline vanadate of the type



100

This solution will be withdrawn and may be subsequently treated by any approved process to recover the values. The ore will next be leached with an acid other than sulfuric and then washed with water. Any

105

suitable acid may be used in this step of the process and it may be either hot or cold. Good results may be obtained with the use of an 8% solution of hydrochloric 5 or nitric acid. This treatment of the ore dissolves the radium content of the ore as radium barium chlorid, (RaBaCl<sub>2</sub>), and the resultant solution may be subsequently treated in any approved manner to recover 10 the radium. The ore may be finally leached with sulfuric acid (preferably a 10% solution) to dissolve any vanadium (as ranadyl sulfate) remaining in the ore. The vanadium solution thus obtained may, if 15 desired, be subsequently treated to recover the vanadium.

In the diagrammatical illustration of the process, shown in the drawing, the various steps of the process are indicated by the reference characters *a*, *b*, *c*, *d*, *e*, *f*, *g*, *h*, *i*, *j*, 20 and the products of the steps involving chemical action are also indicated.

Having fully described my invention, what I claim as new and desire to secure by 25 Letters Patent is:

1. The herein described process of extracting values from carnotite ores, consisting in reducing the ore to a comminuted condition, treating the ore to decompose the barium 30 sulfate, washing the ore to remove the sulfate, leaching the ore with acid to dissolve

the radium content of the ore, and recovering a solution of radium salts.

2. The herein described process of extracting values from carnotite ores, consisting in 35 reducing the ore to a comminuted condition, treating the ore with a solution containing alkaline hydroxid, recovering the resultant alkaline vanadate solution, neutralizing the ore with acid other than sulfuric acid, treat- 40 ing the ore with a heated alkaline carbonate, and recovering a solution of uranium, washing the ore, and leaching the ore with an acid and recovering a radium solution.

3. The herein described process of extracting values from carnotite ores, consisting in 45 reducing the ore to a comminuted condition, treating the ore with a solution containing alkaline hydroxid, recovering the resultant alkaline vanadate solution, treating the ore 50 with a heated alkaline carbonate, and recovering a solution of uranium, washing the ore, and leaching the ore with an acid and recovering a radium solution.

In testimony whereof, I have signed this 55 specification in the presence of two subscribing witnesses.

WARREN F. BLEECKER.

Witnesses:

JOS. A. KELLY,  
HARRY A. KRAELING.